

1

**3,814,679**  
**PREPARATION OF FUELS FOR SUPERSONIC**  
**AIRCRAFT**

Robert Erlmeier, Munich, Friedrich Hilberath, Walberg, Ewald Meisenburg, Wesseling, and Gunter Spengler, Munich, Germany, assignors to Union Rheinische Braunkohlen Kraftstoff Aktiengesellschaft, Wesseling, near Cologne, Germany

No Drawing. Continuation-in-part of abandoned application Ser. No. 88,204, Nov. 9, 1970. This application Mar. 13, 1972, Ser. No. 234,313

Claims priority, application Germany, Nov. 14, 1969,

P 19 57 206,6

Int. Cl. C10l 1/04; C07c 5/04

U.S. Cl. 208—15

5 Claims

## ABSTRACT OF THE DISCLOSURE

Fuels for supersonic aircraft prepared by oligomerizing C<sub>3</sub> and C<sub>4</sub> hydrocarbons which are first made free of isobutylene and hydrogenating the oligomerizates.

## CROSS-REFERENCE TO RELATED APPLICATION

This application is a continuation-in-part of our co-pending application Ser. No. 88,204 filed Nov. 9, 1970 and now abandoned.

## BACKGROUND OF THE INVENTION

This invention relates to a process for the production of fuels for aircraft suitable for supersonic flight, even at speed in excess of Mach 3.

Apart from some exceptional instances, hydrocarbon fuels, which must be available in large quantities, are generally used for supersonic aircraft for economic reasons. The fuels are usually mixtures of representatives of all classes of hydrocarbons, the proportion and constitution of the individual types of hydrocarbon being governed to a large extent both by the origin and by the processing of the starting material. The conditions prevailing during high-velocity supersonic flight impose considerable thermal stresses on the fuels so that, besides satisfying other requirements such as calorific value, vapor pressure and low-temperature behaviour etc., the fuels used for this purpose must show high thermal stability. Most olefins show low thermal or thermooxidation stability, whilst aromatic hydrocarbons show a pronounced tendency to form carbon black because of their unfavorable carbon-hydrogen ratio. On the other hand, normal paraffins have to be separated from the mixtures in order to provide the requisite low-temperature behaviour. Accordingly, supersonic fuels should comprise olefin-free mixtures of predominantly isoparaffins.

Energy content and combustion behaviour are also factors of considerable importance. High calorific value per litre is generally of advantage because considerable distances can then be flown for a given tank volume. It is, however, possible to increase the calorific value per litre only to a limited extent, by employing fuels of higher specific gravity, because this involves deterioration of the low-temperature behaviour and/or combustion behaviour. Combustion behaviour can be regarded as satisfactory when high combustion is obtained with limited thermal radiation and limited soot formation. The smoke point and luminometer number are used for assessment on a laboratory scale. The luminometer number is becoming increasingly more important. It increases with decreasing flame radiation, i.e. decreasing formation of carbon particles in the flame, and should be as high as possible.

Depending upon the type of aircraft and the purpose for which it is to be used, the properties of the fuel have to be adapted to one another in regard to the requirements imposed on thermal stability, combustion behaviour (e.g. luminometer number and smoke point) and the energy

2

content (calorific value per litre) on the one hand, and satisfactory low-temperature behaviour (e.g. freezing point and viscosity) on the other hand. Thus, it has already been proposed to prepare isoparaffinic products having properties suitable for driving jet engines by oligomerizing C<sub>3</sub>—C<sub>4</sub> olefin mixtures and then hydrogenating the oligomers. Since hardly any normal paraffins are present in the products obtained in this way, there is no need for an additional treatment to adjust the necessary low-temperature behaviour. However, the products obtained are not satisfactory to such an extent that they can be used as supersonic fuels.

## SUMMARY OF THE INVENTION

15 It has now been found that especially valuable fuels for supersonic aircraft are obtained if the olefinic C<sub>3</sub>- and C<sub>4</sub>-hydrocarbons chosen for the oligomerization and hydrogenation are first made substantially free of isobutylene.

## DESCRIPTION OF THE INVENTION

The present invention provides a process for the production of fuels for supersonic aircraft which comprises oligomerizing an olefin-containing, C<sub>4</sub>- or C<sub>3</sub>/C<sub>4</sub>-hydrocarbon mixture with a low content of isobutylene, and hydrogenating the resulting oligomer in known manner.

It is an important feature of this new method that the olefin-containing C<sub>4</sub>- and C<sub>3</sub>/C<sub>4</sub>-hydrocarbon mixtures used as starting materials be substantially free from isobutylene, before they are oligomerized and then hydrogenated in the usual way. The supersonic fuels thus obtained exhibit optimum properties if the isobutylene content of the C<sub>4</sub>-hydrocarbons introduced into the oligomerization reactor is at a minimum. Therefore, it is of particular advantage if the isobutylene content does not exceed about 2% by weight based on the C<sub>4</sub>-olefins and preferably does not exceed about 1%. Although higher proportions of isobutylene may be tolerated, they should preferably remain below 10% by weight. The oligomerizates thus obtained are not only useful as supersonic fuels as such but also as mixing components. For example, valuable supersonic fuels may be obtained by mixing according to the invention the hydrogenated oligomerizates with properly refined and hydrogenated straight-run fractions of crude oils having a corresponding boiling range, e.g. 190–250° C. The proportions of the said fractions which can be admixed increase with improvement in the properties of the oligomerizates, i.e. with the lowering of the isobutylene content in the hydrocarbon mixture before oligomerization.

The removal of the isobutylene may be conducted in known manner. For example, the isobutylene can be extracted from a C<sub>4</sub>-hydrocarbon mixture at ambient temperature, utilizing a 50 percent sulfuric acid as a solvent. 55 The hydrocarbon phase is separated, neutralized and washed with water and then used as feed stock for oligomerization. The isobutylene may be separated from the acid phase at high temperatures and under a low pressure. On the other hand, the isobutylene may be selectively oligomerized in the fluid phase at a temperature of about 100° C. and under a slightly elevated pressure, for example in the presence of a noble metal catalyst. The di-isobutylenes and tri-isobutylenes thus obtained can be separated from the other olefines by distillation. In this way up to 99% of the isobutylene are removed from the C<sub>4</sub>-hydrocarbon mixture.

After the removal of the isobutylene, the olefin-containing C<sub>4</sub>- and C<sub>3</sub>/C<sub>4</sub>-hydrocarbon mixtures ordinarily are oligomerized in contact with an acidic oligomerization catalyst such as phosphoric acid supported on an inert carrier such as kieselguhr. When using this catalyst the oligomerization is usually conducted at a temperature be-

tween about 125 and 260° C. at an elevated pressure, e.g. 15 atm.

The hydrogenation of the oligomerizes thus obtained is conducted in known manner in the presence of a suitable hydrogenation catalyst such as platinum, ruthenium, nickel and the oxides or sulfides of molybdenum, tungsten etc. These materials may be supported by silica-alumina, kieselguhr and the like. Usually the hydrogenation is conducted at a temperature of up to about 450° C. and under a pressure of up to about 200 atm.

Fuels obtained in this manner have particularly valuable properties, for example especially high thermo-oxidation stability, and they are superior to fuels prepared from oligomers obtained in a similar conventional manner from starting materials which had not been freed from isobutylene.

A further improvement in the fuels can be obtained by removing the aromatic hydrocarbons formed in small quantities, for example by hydrogenating them together with the olefinic hydrocarbons in known manner as de-

The following parameters were determined in order to evaluate the various fuels:

- A. Thermo-oxidation stability in accordance with ASTM D 873 by aging 100 ml. of fuel for 5 hours at 148.9° C. (300° F.) under an oxygen pressure of 7 atms. (100 p.s.i.), and then determining the potential residue as a measure of stability.
- B. Low-temperature behaviour by measuring (i) the crystallization point in accordance with DIN 51,782, and (ii) the low-temperature viscosity at -34.4° C. in accordance with DIN 51,562.
- C. Energy behaviour by determining the lower calorific value.
- D. Combustion behaviour by measuring (i) the luminometer number in accordance with ASTM D 1740-67 T, and (ii) the smoke point in accordance with ASTM D 1322-64.

The results with these four different fuels are set out below in the table.

TABLE

| Fuel        | Boiling range, ° C. | A           |         | B        |           | C        |    | D       |  |
|-------------|---------------------|-------------|---------|----------|-----------|----------|----|---------|--|
|             |                     | Mg./100 ml. | I, ° C. | II, cst. | Keal./kg. | Keal./l. | I  | II, mm. |  |
| <b>I:</b>   |                     |             |         |          |           |          |    |         |  |
| a.....      | 193-210             | 10.6        | <-80    | 10.62    | 10,485    | 8,261    | 64 | 33      |  |
| b.....      | 220-239             | 34.1        | <-80    | 34.68    | 10,480    | 8,435    | 59 | 30      |  |
| c.....      | 241-251             | 51.4        | <-80    | 86.99    | 10,460    | 8,556    | 54 | 27      |  |
| <b>II:</b>  |                     |             |         |          |           |          |    |         |  |
| a.....      | 193-217             | 4.1         | <-80    | 13.44    | 10,515    | 8,212    | 80 | 40      |  |
| b.....      | 205-236             | 10.5        | <-80    | 30.98    | 10,565    | 8,462    | 70 | 35      |  |
| c.....      | 239-272             | 25.4        | <-60.5  | 12.24    | 10,425    | 8,507    | 65 | 31      |  |
| <b>III:</b> |                     |             |         |          |           |          |    |         |  |
| a.....      | 194-218             | 7.3         | <-80    | 12.55    | 10,500    | 8,234    | 73 | 35      |  |
| b.....      | 214-232             | 17.0        | <-80    | 25.24    | 10,490    | 8,360    | 74 | 34      |  |
| c.....      | 231-274             | 33.1        | <-80    | 69.90    | 10,415    | 8,467    | 63 | 34      |  |
| <b>IV:</b>  |                     |             |         |          |           |          |    |         |  |
| a.....      | 194-210             | 4.0         | <-55.5  | 10.39    | 10,520    | 8,253    | 88 | 47      |  |
| b.....      | 205-233             | 9.0         | <-38.5  | 20.24    | 10,490    | 8,308    | 81 | 43      |  |

scribed above. In addition to isoparaffins, the fuel thus obtained contains a small proportion of naphthenes.

It is also possible initially to subject the oligomer to a mild selective hydrogenation i.e. at ambient temperature and under a pressure of about 30 to 50 atm. in the presence of a catalyst containing a noble metal as the catalytic material in order to saturate the olefins. The aromatic hydrocarbons are then removed from the product in known manner, for example by extractive distillation. The extraction may be conducted for example by an aqueous solution of an organic solvent such as N-methyl-pyrrolidone at ambient or near ambient temperature in a tower type extractor followed by processing the extract phase and the raffinate phase in known manner.

If desired the product can be subjected to stronger hydrogenation to give a fuel free from aromatic hydrocarbons and naphthenes. These products, which consist almost entirely of isoparaffinic hydrocarbons, have a particularly high thermostability. In some instances it can be of advantage for the starting product to have a high propylene content. The usual additives can of course be added to the fuels.

#### EXAMPLE

Several fuels were prepared in known manner as described by oligomerization and hydrogenation:

Fuel I from a C<sub>4</sub>-hydrocarbon mixture containing 37.8% by weight of isobutylene,

Fuel II from an isobutylene-free C<sub>4</sub>-hydrocarbon mixture, Fuel III from C<sub>3</sub>/C<sub>4</sub>-hydrocarbon mixture containing 31.3% by weight of propylene and 23.5% by weight of isobutylene, and

Fuel IV from a C<sub>3</sub>/C<sub>4</sub>-hydrocarbon mixture containing 82.8% by weight of propylene and 7.4% by weight of isobutylene.

What we claim is:

1. In a process for the production of fuels for supersonic aircrafts by oligomerizing an olefin-containing C<sub>4</sub> or C<sub>3</sub>/C<sub>4</sub> hydrocarbon mixture which contains isobutylene and hydrogenating the resulting oligomer, the improvement which comprises removing the isobutylene contained in the hydrocarbon mixture to less than 10% by weight based on the C<sub>4</sub>-olefins before oligomerizing.
2. In a process for the production of fuels for supersonic aircraft by oligomerizing an olefin-containing C<sub>4</sub> or C<sub>3</sub>/C<sub>4</sub> hydrocarbon mixture which contains isobutylene and hydrogenating the resulting oligomer, the improvement which comprises removing the isobutylene contained in the hydrocarbon mixture to less than 2% by weight based on the C<sub>4</sub>-olefins before oligomerizing.
3. In a process according to claim 1, the improvement which comprises hydrogenating the oligomer selectively to saturate the olefins and removing the aromatic hydrocarbons from the oligomer by extractive distillation.
4. Fuel components for supersonic aircraft produced according to the process of claim 1.
5. Fuel components for supersonic aircraft produced according to the process of claim 3.

#### References Cited

##### UNITED STATES PATENTS

65 3,125,503 3/1964 Kerr et al. 208—15

##### OTHER REFERENCES

Bachman, Preprints of the American Chemical Society, Division of Petroleum Chemistry, vol. 5, No. 4, September 1960, New York, N.Y., pp. C-39 to C-48.

HERBERT LEVINE, Primary Examiner

U.S. Cl. X.R.

75 260—683.15 R, 683.9